

## UNITED STATES PATENT OFFICE

ERNST GALLE, OF LUDWIGSHAFEN-ON-THE-RHINE, AND HERMANN ZORN, OF MANNHEIM, GERMANY, ASSIGNORS TO I. G. FARBENINDUSTRIE AKTIENGESELLSCHAFT, OF FRANKFORT-ON-THE-MAIN, GERMANY, A CORPORATION OF GERMANY

PROCESS FOR THE CONVERSION OF HYDROCARBONS OF HIGH BOILING POINT INTO OTHERS OF LOW BOILING POINT

No Drawing. Application filed December 19, 1928, Serial No. 327,179, and in Germany February 4, 1928.

It is already known that phosphoric acids are capable of splitting hydrocarbons of high molecular weight, such as mineral oils or tar oils into such of lower molecular weight at elevated temperatures.

We have now found that a substantially better splitting action is exerted by a catalyst consisting of or containing a salt of metaphosphoric acid, especially the heavy-metal salts of the said acid and in particular the metaphosphates of the metals of the sixth group of the periodic system. The preferred method of operating consists in passing the vaporized hydrocarbons over the catalyst in association with inert gases such as nitrogen at elevated temperatures and, when found desirable, under pressure. The catalyst may be attached to a carrier, such as pumice, silica gel or the like, upon which the salt, or mixture of different salts of phosphoric acids is deposited.

In addition to hydrocarbons of low boiling point, considerable amounts of unsaturated gaseous hydrocarbons such as ethylene, propylene and butylene are usually obtained.

The cracking process is carried out under otherwise known conditions and usually between about 400° and 800° C. Inert gases such as nitrogen or carbon dioxide may also be added or also hydrogen. If desired, the process may also be carried out under pressure of say up to 50 atmospheres. The said cracking process may be carried out either in the liquid or gaseous phase as required.

The following examples will further illustrate the nature of this invention which however is not restricted thereto. The parts are by weight.

40 *Example 1*

100 parts of brown coal tar in a vaporized form, are passed at 600° centigrade over a catalyst composed of uranyl metaphosphate deposited on pumice. 35 parts of benzene hydrocarbons boiling below 200° centigrade are obtained, together with 20 parts of cracked gases containing 35 per cent of olefines. The residue consists of oil boiling above 200° centigrade and free from coke.

Example 2

100 parts of crude mineral oil in vaporized form are passed at 580° centigrade and in the presence of nitrogen, over a catalyst composed of chromium metaphosphate, 40 parts of a product boiling below 200° centigrade are obtained, and 18 parts of cracked gases which to the extent of about one-third consist of olefines. The residue is an oil boiling above 200° centigrade and free from coke.

What we claim is:—

1. In the process of splitting hydrocarbons of high molecular weight into such of lower molecular weight by the action of heat, the step of carrying out the said treatment in the presence of a catalyst comprising a salt of metaphosphoric acid at a temperature high enough to promote the conversion.

2. In the process of splitting hydrocarbons of high molecular weight into such of lower molecular weight by the action of heat, the step of passing the said hydrocarbons of high molecular weight over a catalyst comprising a salt of metaphosphoric acid at a temperature high enough to promote the conversion.

3. In the process of splitting hydrocarbons of high molecular weight into such of lower molecular weight by the action of heat, the step of vaporizing the said hydrocarbons of high molecular weight and passing them over a catalyst comprising a salt of metaphosphoric acid at a temperature high enough to promote the conversion.

4. In the process of splitting hydrocarbons of high molecular weight into such of lower molecular weight by the action of heat, the step of vaporizing the said hydrocarbons of high molecular weight and passing them in association with inert gases over a catalyst comprising a salt of metaphosphoric acid at a temperature high enough to promote the conversion.

5. In the process of splitting hydrocarbons of high molecular weight into such of lower molecular weight by the action of heat, the step of carrying out the said treatment in the presence of a catalyst comprising a heavy metal salt of metaphosphoric acid at a temperature high enough to promote the conversion.

6. In the process of splitting hydrocarbons of high molecular weight into such of lower molecular weight by the action of heat, the step of passing the said hydrocarbons of high molecular weight over a catalyst comprising a heavy metal salt of metaphosphoric acid at a temperature high enough to promote the conversion.

7. In the process of splitting hydrocarbons of high molecular weight into such of lower molecular weight by the action of heat, the step of vaporizing the said hydrocarbons of high molecular weight and passing them over a catalyst comprising a heavy metal salt of metaphosphoric acid at a temperature high enough to promote the conversion.

8. In the process of splitting hydrocarbons of high molecular weight into such of lower molecular weight by the action of heat, the step of vaporizing the said hydrocarbons of high molecular weight and passing them in association with inert gases over a catalyst comprising a heavy metal salt of metaphosphoric acid at a temperature high enough to promote the conversion.

9. In the process of splitting hydrocarbons of high molecular weight into such of lower molecular weight by the action of heat, the step of vaporizing the said hydrocarbons of high molecular weight and passing them at a temperature of about 400° to 800° C. over a catalyst comprising a salt of metaphosphoric acid.

10. In the process of splitting hydrocarbons of high molecular weight into such of lower molecular weight by the action of heat, the step of vaporizing the said hydrocarbons of high molecular weight and passing them at a temperature of about 400° to 800° C. over a catalyst comprising a metaphosphate of a metal from the sixth group of the periodic system.

11. A process for cracking a mineral oil, which comprises vaporizing and passing the said mineral oil over a catalyst comprising chromium metaphosphate at a temperature high enough to promote the conversion.

In testimony whereof we have hereunto set our hands.

50

ERNST GALLE.  
HERMANN ZORN.

55

60

65